

1

3,183,189  
PETROLEUM LUBRICANTS STABILIZED WITH  
BACTERICIDES

Edward B. Hodge, Terre Haute, Ind., assignor to Commercial Solvents Corporation, New York, N.Y., a corporation of Maryland  
No Drawing. Filed Mar. 20, 1961, Ser. No. 96,695  
16 Claims. (Cl. 252—49.5)

My invention relates to a stabilized petroleum lubricant and more particularly to a process for the production of stabilized petroleum lubricants containing as the active stabilizing agent nitroamines having the structural formula:



where R is selected from the group consisting of lower alkyl and hydrogen; where R<sub>1</sub> is a member selected from the group consisting of —N(R<sub>2</sub>)<sub>2</sub>, morpholino, and piperidyl; and where R<sub>2</sub> is a member selected from the group consisting of hydrogen, tetrahydrofurfuryl, lower alkyl, and lower hydroxyalkyl.

It is well known that organisms from the groups consisting of *Corynebacterium*, *Achromobacter*, *Pseudomonas*, *Nocardia* and *Mycobacterium* metabolize petroleum hydrocarbons and fatty acids and thereby produce undesirable oxidation products.

The petroleum industry has long been interested in the stabilization of various petroleum products such as cutting oils, hydraulic fluids, etc., against breakdown by bacteria which metabolize the hydrocarbons with the concurrent formation of deleterious metabolites.

Many compounds have been used as stabilization agents in lubricants, but very few have been found to be commercially successful due to the fact that the compounds are unstable, or are not active against a wide variety of microorganisms.

Among the nitroamines having the above structural formula are included N-(2-nitroisobutyl)diisopropylamine, N-(2-nitropropyl)morpholine, N-(2-nitropropyl)diethylamine, N-(2-nitropropyl)diisobutylamine, N-(2-nitrobutyl)dimethylamine, N-(2-nitrobutyl)-2-ethylhexylamine, N-(2-nitrobutyl)-1-amino-2-propanol, N-(2-nitrobutyl)morpholine, N-(2-nitrobutyl)piperidine, N-(2-nitrobutyl)tetrahydrofurfurylamine, etc. I have found that in some instances I can obtain total inhibition of bacterial growth in petroleum lubricants at concentrations as low as 100 p.p.m. I prefer to include at least 1,000 p.p.m. in most petroleum formulations. However, I can employ amounts up to about 2% by weight of the active nitroamines when the latter is soluble to this extent in the particular petroleum hydrocarbon composition.

I have found that my active ingredients are effective bacteriostatic agents in petroleum containing lubricants such as cutting oils, penetrating oils, grinding lubricants, iron tinning lubricants, core oils, hydraulic fluids, etc.

The following examples set out lubricating compositions in which my active ingredients act as effective bacteriostatic agents. It is not intended that my invention be limited to the compositions, portions, or lubricants set out below; but rather I intend for all equivalents and variations obvious to those skilled in the art to be included within the scope of this specification and the attached claims.

### EXAMPLE I

To test the use of my active ingredients in cutting oils, a 25:1 water-cutting oil emulsion was prepared. The cutting oil concentrate used was a proprietary cutting oil containing no bacteria inhibitors such as that sold by

2

Texaco Incorporated under the name of Soluble Oil Texaco-C. To each of one-gallon containers was added 1 liter of water-cutting oil emulsion. Desired amounts of my nitroamines were added to the cutting-oil emulsion in the first container. No inhibitor was added to the other container which was used as a control. At the beginning of the experiment, each unit was inoculated with 5 mls. of a heterogeneous bacterial culture which had grown for several years in a water-cutting oil emulsion. Aeration and mixing were obtained by using an air lift to continually circulate the mixture. The test was continued for a period of six weeks and during the six-week period, 5 mls. of bacterial culture were added at periodic weekly intervals.

15 The following table sets out the results of the above tests and the number of days of bacterial inhibition when the described concentration of the desired nitroamines were incorporated into the cutting-oil emulsion.

Table I

| Nitroamine                              | Concentration in 25:1 Water-Cutting Oil Emulsion | Number of Days Effective |
|-----------------------------------------|--------------------------------------------------|--------------------------|
| N-(2-nitroisobutyl)diethylamine         | 1,000                                            | >42                      |
| N-(2-nitropropyl)morpholine             | 1,000                                            | >42                      |
| N-(2-nitropropyl)diethylamine           | 1,000                                            | 21                       |
| N-(2-nitropropyl)diisobutylamine        | 1,000                                            | >21                      |
| N-(2-nitrobutyl)dimethylamine           | 1,000                                            | >42                      |
| N-(2-nitrobutyl)-2-ethylhexylamine      | 1,000                                            | 10                       |
| N-(2-nitrobutyl)-1-amino-2-propanol     | 1,000                                            | 14                       |
| N-(2-nitrobutyl)morpholine              | 1,000                                            | 35                       |
| N-(2-nitrobutyl)piperidine              | 500                                              | 14                       |
| N-(2-nitrobutyl)tetrahydrofurfurylamine | 1,000                                            | >42                      |
| Control                                 | 1,000                                            | 10                       |
|                                         |                                                  | 0                        |

### EXAMPLE II

The following is a water emulsifiable cutting oil which is adequately protected by 1,000 p.p.m. of my nitroamine inhibitors:

|                   | Percent by weight |
|-------------------|-------------------|
| Light mineral oil | 90                |
| Oleic acid        | 10                |

### EXAMPLE III

The following is a stabilized steam cylinder oil which is adequately protected by 1,000 p.p.m. of N-(2-nitrobutyl)dimethylamine.

|                        | Percent |
|------------------------|---------|
| S.A.E. lubricating oil | 90      |
| Oleic acid             | 10      |

### EXAMPLE IV

The following is a core oil which is adequately protected by 1,000 p.p.m. of N-(2-nitrobutyl)morpholine.

|                                     | Percent |
|-------------------------------------|---------|
| Crude tall oil                      | 25      |
| Fuel oil                            | 35      |
| Tall oil ester (glycol or glycerol) | 40      |

### EXAMPLE V

The following is a cutting oil which is adequately protected by 1,000 p.p.m. of N-(2-nitrobutyl)piperidine.

|                   | Percent |
|-------------------|---------|
| Tallow            | 65      |
| Paraffin wax      | 29      |
| Beeswax           | 1.3     |
| Oxalic acid       | 1.3     |
| Potassium citrate | 1.3     |
| Urea              | 0.4     |

Now having described my invention, what I claim is:

1. A liquid petroleum composition consisting essentially of a liquid petroleum lubricant hydrocarbon and a sufficient amount of N-(2-nitroisobutyl)diisopropylamine to stabilize said hydrocarbon against metabolizing bacteria.

2. A liquid petroleum composition consisting essentially of a liquid petroleum lubricant hydrocarbon and a sufficient amount of N-(2-nitropropyl)morpholine to stabilize said hydrocarbon against metabolizing bacteria.

3. A liquid petroleum composition consisting essentially of a liquid petroleum lubricant hydrocarbon and a sufficient amount of N-(2-nitropropyl)diisopropylamine to stabilize said hydrocarbon against metabolizing bacteria.

4. A liquid petroleum composition consisting essentially of a liquid petroleum lubricant hydrocarbon and a sufficient amount of N-(2-nitropropyl)diisobutylamine to stabilize said hydrocarbon against metabolizing bacteria.

5. A liquid petroleum composition consisting essentially of a liquid petroleum lubricant hydrocarbon and a sufficient amount of N-(2-nitrobutyl)dimethylamine to stabilize said hydrocarbon against metabolizing bacteria.

6. A liquid petroleum composition consisting essentially of a liquid petroleum lubricant hydrocarbon and a sufficient amount of N-(2-nitrobutyl)-2-ethylhexylamine to stabilize said hydrocarbon against metabolizing bacteria.

7. A liquid petroleum composition consisting essentially of a liquid petroleum lubricant hydrocarbon and a sufficient amount of N-(2-nitrobutyl)-1-amino-2-propanol to stabilize said hydrocarbon against metabolizing bacteria.

8. A liquid petroleum composition consisting essentially of a liquid petroleum lubricant hydrocarbon and a sufficient amount of N-(2-nitrobutyl)morpholine to stabilize said hydrocarbon against metabolizing bacteria.

9. A liquid petroleum composition consisting essentially of a liquid petroleum lubricant hydrocarbon and a sufficient amount of N-(2-nitrobutyl)piperidine to stabilize said hydrocarbon against metabolizing bacteria.

10. A liquid petroleum composition consisting essentially of a liquid petroleum lubricant hydrocarbon and a sufficient amount of N-(2-nitrobutyl)tetrahydrofurfurylamine to stabilize said hydrocarbon against metabolizing bacteria.

11. An aqueous petroleum emulsion consisting essentially of an aqueous petroleum lubricant hydrocarbon emulsion and a sufficient amount of a nitroamine to stabilize said hydrocarbon against metabolizing bacteria, said nitroamine having the structural formula:



where R is selected from the group consisting of lower alkyl and hydrogen; where R<sub>1</sub> is a member selected from the group consisting of —N(R<sub>2</sub>)<sub>2</sub>, morpholino, and piperidyl; and where R<sub>2</sub> is a member selected from the group consisting of hydrogen, tetrahydrofurfuryl, lower alkyl, and lower hydroxyalkyl.

12. A liquid petroleum composition consisting essentially of a liquid petroleum lubricant hydrocarbon and a sufficient amount of a nitroamine to stabilize said hydrocarbon against metabolizing bacteria, said nitroamine having the structural formula:



where R is selected from the group consisting of lower alkyl and hydrogen; where R<sub>1</sub> is a member selected from the group consisting of —N(R<sub>2</sub>)<sub>2</sub>, morpholino, piperidyl; and where R<sub>2</sub> is a member selected from the group consisting of hydrogen, tetrahydrofurfuryl, lower alkyl and lower hydroxyalkyl.

13. The composition of claim 12 wherein the composition contains from about 100 p.p.m. to 2% by weight of the nitroamine.

14. The composition of claim 11 wherein the composition contains from about 100 p.p.m. to 2% by weight of the nitroamine.

15. The composition of claim 11 wherein the composition is a cutting oil.

16. The composition of claim 11 wherein the composition is a steam cylinder oil.

35 **References Cited by the Examiner**  
**UNITED STATES PATENTS**

|           |       |                |       |           |
|-----------|-------|----------------|-------|-----------|
| 2,419,506 | 4/47  | Senkus         | ----- | 260—583   |
| 2,465,958 | 3/49  | Senkus         | ----- | 260—347.7 |
| 2,474,791 | 6/49  | Senkus         | ----- | 260—247   |
| 2,588,428 | 3/52  | Stewart et al. | ----- | 167—22    |
| 2,812,332 | 11/57 | Pennino        | ----- | 167—33    |
| 2,913,414 | 11/59 | Hodge          | ----- | 252—51.5  |
| 3,054,749 | 9/62  | Bennett et al. | ----- | 252—8.55  |

40 **FOREIGN PATENTS**

|            |      |            |
|------------|------|------------|
| 107,419    | 5/39 | Australia. |
| 160,367    | 1/55 | Australia. |
| 50 421,189 | 3/47 | Italy.     |

DANIEL E. WYMAN, Primary Examiner.

JULIUS GREENWALD, Examiner.